

Oct. 29, 1935.

F. F. FOWLE ET AL

2,019,447

OVERHEAD ELECTRIC TRANSMISSION LINE

Filed Jan. 8, 1934

Overhead Electric Transmission Line,  
of Carbon-Steel Conductors Desirably Hypoeutectoid,  
Containing At Least 0.25% C, Not In Excess of 0.30% Mn,  
and Desirably Not In Excess of 0.15% Si.



Inventors

By

FRANK F. FOWLE AND  
FREDERICK M. CRapo,  
Schley & Tracy  
Attorneys

## UNITED STATES PATENT OFFICE

2,019,447

## OVERHEAD ELECTRIC TRANSMISSION LINE

Frank F. Fowle, Winnetka, Ill., and Frederick M. Crapo, Muncie, Ind., assignors to Indiana Steel & Wire Company, Muncie, Ind., a corporation of Indiana

Application January 8, 1934, Serial No. 705,830

4 Claims. (Cl. 173—13)

Our invention relates to overhead electric transmission lines using ferrous conductors, with particular reference to A. C. transmission lines although our invention is not limited to A. C. lines. Our invention is applicable, for instance, for power lines, telephones lines, telegraph lines, signal lines, etc., and is of especial value for telephone transmission lines; and the conductors involved may be not only the wires of the transmission circuit proper, but also include various ancillary conductors, such as ground wires, shield wires, messenger cables, catenary supports, etc., which may be primarily for other than conducting purposes and/or may actually serve to conduct current only occasionally. Therefore, by the term "overhead electric transmission line" we mean an overhead line which has a series of wire-spans under tension and which may be required to carry electric current; and by the terms "ferrous conductor" or "carbon-steel conductor" we mean a conductor which may be required to serve as a current-carrier for an electrical system and of which the cross-section is mainly of ferrous material, specifically carbon steel in our invention, and any coating (as of zinc or copper) is a relatively small part of the cross-section. The term "carbon steel" is used in its accepted sense, (as shown by "The Making, Shaping, and Treating of Steel", by Camp and Francis, published by the Carnegie Steel Company, Fourth Edition, pages 259 and 707, generally accepted as authoritative), as meaning steels in which carbon is the element fundamentally employed to control physical properties; and in which manganese is less in amount than about 1.0%, although in previous hypoeutectoid carbon steels it has usually been greater in amount than the carbon. It is the object of our invention to produce a transmission line of carbon-steel conductor (un-coated or coated as with zinc or copper) which has its tensile strength and its electrical conductivity both relatively high. Generally in the prior art an increase in tensile strength in ferrous conductors has been obtained at the cost of decreased electrical conductivity, and an increase in electrical conductivity at the cost of decreased tensile strength; but by our invention we are able to get both relatively high. The accompanying drawing illustrates our invention diagrammatically. The single figure of such drawing is a diagrammatic view of an overhead electric transmission line, of ferrous conductor, in accordance with our invention, the particular

character of ferrous conductor being indicated by a legend on the drawing.

Heretofore the ferrous conductors in general use for telephone, telegraph, and signal lines and in some instances for power lines, have been of three general commercial grades known as "E. B. B." (extra best best), "B. B." (best best), and "steel". Approximate tensile strengths and D. C. resistivities of these grades are as follows:

| Grade    | Approximate D. C. resistivity in ohms per mile-pound | Approximate tensile strength in pounds per square inch | 10 |
|----------|------------------------------------------------------|--------------------------------------------------------|----|
| E. B. B. | 4850                                                 | 45,000                                                 | 13 |
| B. B.    | 5800                                                 | 51,000                                                 |    |
| Steel.   | 6750                                                 | 55,000                                                 |    |

Three other commercial grades of ferrous conductors have also heretofore been used in some instances for power lines; especially for overhead ground wires and/or shield wires, and for long spans such as wide river crossings. These other three grades are commonly known as "Siemens-Martin", "high strength", and "extra-high strength", and named in the order of increasing tensile strength and D. C. resistivity. Approximate tensile strengths and D. C. resistivities of these three grades are as follows:

| Grade               | Approximate D. C. resistivity in ohms per mile-pound | Approximate tensile strength in pounds per square inch | 30 |
|---------------------|------------------------------------------------------|--------------------------------------------------------|----|
| Siemens-Martin      | 7280                                                 | 90,000                                                 | 35 |
| High strength       | 8320                                                 | 149,000                                                |    |
| Extra-high strength | 9360                                                 | 200,000                                                |    |

Special grades of ferrous conductors having still higher tensile strength and often higher electrical resistivity are known as "high strength crucible" and "extra-high strength plow"; but these two grades are used infrequently, or only under some very unusual conditions, as for an exceptionally long power span where the highest attainable wire-strength is an imperative requirement regardless of other considerations.

In all the grades known as "Siemens-Martin", "high strength", "extra strength", "high strength crucible", and "extra-high strength plow", the advantages of increased tensile strength have been obtained at the sacrifice of electrical conductivity; so that while the tensile strengths of such grades are substantially great-

er than those of "E. B. B.", "B. B.", or "steel", above mentioned, their electrical conductivities are substantially less. Such increased tensile strengths have been obtained fundamentally by making the wires of steels which have high contents of carbon, and/or to some extent and in some cases by heat treatment and/or by cold-working the material in the process of wire drawing.

In the high-carbon ferrous conductors of the prior art of overhead transmission, however, the high carbon content has been accompanied by a high content of manganese. This manganese content has usually exceeded the carbon content, and often exceeded it very substantially; and has contributed somewhat to the increase in tensile strength in the five higher-strength grades above considered. But it has contributed more considerably to the increase in D. C. resistivity in these higher-strength grades; for while such increase in D. C. resistivity has been due in some measure to the content of carbon, it has been due in still greater measure to the content of manganese.

This situation is due to the fact that the addition of carbon to a low-carbon steel of the prior art increases its tensile strength in a proportionately greater degree than the addition of an equal amount of manganese, but increases its D. C. resistivity in a proportionately less degree than the addition of an equal amount of manganese; and that the elimination of manganese in a medium-carbon or high-carbon steel such as has been used in the prior art decreases its tensile strength in proportionately less degree than the elimination of an equal amount of carbon, but decreases its D. C. resistivity in proportionately greater degree than the elimination of an equal amount of carbon.

Heretofore high manganese has in general been assumed to be necessary in any medium-carbon and higher-carbon steels used in transmission lines, for various reasons and especially for cleansing the steel in the process of manufacture; and its effect in increasing the D. C. resistivity, if considered at all, either was deemed not seriously objectionable or was considered unavoidable.

In contradistinction to the practice of the prior art, in which increased tensile strength has apparently inevitably been accompanied by an increase in D. C. resistivity, we increase the tensile strength of overhead ferrous conductors without correspondingly increasing the D. C. resistivity. To do this, we take advantage of the relative effects which are producible by carbon and manganese on tensile strength and D. C. resistivity respectively, by using carbon to obtain the desired increase in tensile strength and by restricting the use of manganese and thereby avoiding in large measure the increase in D. C. resistivity.

In carrying out our invention, therefore, we do two fundamental things:

1. We provide a sufficient carbon content in the ferrous conductor so that the tensile strength is high and the skin effect low. As the carbon content of ferrous material is increased, the tensile strength is also increased, and at the same time the magnetic permeability and therefore the skin effect is decreased. There is a bend in the region of 0.25% to 0.30% carbon in the curve showing the relation between carbon content of steel and skin effect, and a marked rise in skin effect as the carbon content decreases below that region; as is shown in Fig. 7 of Patent No.

1,691,869 granted to one of us (Fowle) on November 13, 1928. Advantage is taken of the high tensile strength and the reduction in skin effect by the provision of relatively high carbon (more than 0.30%) in the steel of the conductors of that Fowle Patent No. 1,691,869; and also by the preferred provision of more than 0.25% of carbon in the ferrous conductor (coated or uncoated) of the telephone transmission line forming the subject-matter of the co-pending application of the other of us (Crapo) Serial No. 543,024, filed June 8, 1931, now Patent No. 1,942,411, granted January 9, 1934.

2. We keep relatively low the content of manganese. In every case we keep it below an upper limit of 0.30%, and desirably well below it; for our invention does not require that any manganese be present. As the manganese content is lowered, it becomes possible, when so desired, to increase the carbon content in amounts greater proportionately than the reduction in manganese, without appreciably changing the D. C. resistivity; and thus to increase the tensile strength. There is no lower limit to the manganese content from the stand-point of beneficial effect in lowering the D. C. resistivity.

In addition to these two fundamental things, of high carbon and low manganese, we also preferably keep the silicon content low, desirably below 0.15% as a maximum and as much below that as possible; for the presence of silicon tends markedly to raise the D. C. resistivity, and our invention does not require the presence of any silicon.

Our present invention is thus concerned fundamentally with the carbon content and the manganese content, and secondarily with the silicon content, of the general class of carbon steels. Various other elements which may exist in carbon steels, such as phosphorus and sulphur, may also be present in varying small amounts. These carbon steels may be copper-bearing steels.

Thus our transmission line comprises a carbon-steel conductor (coated or not) which is high in carbon and not high in manganese, and which is desirably low in silicon.

In addition to this matter of the contents of carbon and manganese, and of silicon, we may and preferably do provide certain increases in tensile strength by heat-treatment and/or cold-working. That is, our present invention deals fundamentally with the chemical composition rather than with the grain structure of the carbon-steel conductor involved, and is intended to apply generically to grain structures of whatever sort, whether in annealed state or in some other state such as may be obtained by certain heat treatments and/or by mechanical working.

Such a transmission line has the advantage of high electrical conductivity, for both direct currents and alternating currents, as compared with previous ferrous transmission lines of corresponding carbon contents. It is especially advantageous for alternating or pulsating currents, because of the decreased skin effect due to the high carbon. At the same time, by reason of having the carbon content high, and although having the content of manganese not high, we get high tensile strength. Thus we combine high tensile strength with high conductivity.

The carbon content of our ferrous conductor must be at least 0.25%, and is desirably at least 0.30%. It may be considerably higher; but we find it desirable to keep it below the eutectoid point, of about 0.90%. The manganese content

of our ferrous conductor must not exceed 0.30%. The silicon content should not exceed 0.15%.

An example of carbon-steel conductor used in our invention is a No. 12 B. W. G. galvanized steel wire in which the steel contained approximately 0.41% of carbon, approximately 0.21% of manganese, and less than 0.01% of silicon. A sample of this wire was hot-galvanized after being annealed, and showed a D. C. resistivity of approximately 5360 ohms per mile-pound, and a tensile strength of approximately 74,000 pounds per square inch. Another sample of this wire was hot-galvanized after receiving a heat-treatment and some cold drawing, and showed a D. C. resistivity of 5460 ohms per mile-pound, and a tensile strength of approximately 135,000 pounds per square inch.

Another example of carbon-steel conductor used in our invention is a No. 12 B. W. G. galvanized wire in which the steel contained approximately 0.35% of carbon, approximately 0.20% of manganese, and approximately 0.10% of silicon. A sample of this wire was hot-galvanized after being annealed, and showed a D. C. resistivity of approximately 6000 ohms per mile-pound, and a tensile strength of approximately 72,500 pounds per square inch. Another sample of this wire was hot-galvanized without being annealed, and showed a D. C. resistivity of approximately 6070 ohms per mile-pound, and a tensile strength of approximately 120,000 pounds per square inch.

By building an overhead transmission line of a carbon-steel conductor (coated or uncoated) conforming to the above requirements, it is possible to have both high tensile strength and high electrical conductivity. Such a transmission line

is of value for both alternating and direct currents, and for the transmission of electric power as well as of telephone, signal, and telegraph currents.

It is also advantageous for ground wires, shield wires, messenger cables, catenary supports, etc.; and either as a single wire or in a stranded cable. But it is of special advantage for the transmission of relatively high-frequency currents, such as those used in telephonic transmission; where the frequency is voice frequency, of the order of 100 to 3000 cycles per second, and the currents are usually small, not exceeding about 50 milliamperes.

We claim as our invention:

15

1. An overhead electric transmission line, comprising a carbon-steel conductor which is to carry current and which contains at least 0.25% of carbon and not in excess of 0.30% of manganese.

2. An overhead electric transmission line, comprising a hypoeutectoid carbon-steel conductor which is to carry current and which contains at least 0.25% of carbon and not in excess of 0.30% of manganese.

3. An overhead electric transmission line, comprising a carbon-steel conductor which is to carry current and which contains at least 0.25% of carbon, not in excess of 0.30% of manganese, and not on excess of 0.15% silicon.

4. An overhead electric transmission line, comprising a hypoeutectoid carbon-steel conductor which is to carry current and which contains at least 0.25% of carbon, not in excess of 0.30% of manganese, and not in excess of 0.15% silicon.

FRANK F. FOWLE. 35  
FREDERICK M. CRAPO.

#### CERTIFICATE OF CORRECTION.

Patent No. 2,019,447.

October 29, 1935.

FRANK F. FOWLE, ET AL.

It is hereby certified that error appears in the printed specification of the above numbered patent requiring correction as follows: Page 1, second column, line 26, after "and" insert are; and line 50, for "extra" read extra-high; page 3, first column, line 6, for "0,21%" read 0.21%; and second column, line 29, claim 3, for "on" read in; and that the said Letters Patent should be read with these corrections therein that the same may conform to the record of the case in the Patent Office.

Signed and sealed this 21st day of January, A. D. 1936.

Seal)

Leslie Frazer  
Acting Commissioner of Patents.

of our ferrous conductor must not exceed 0.30%. The silicon content should not exceed 0.15%.

An example of carbon-steel conductor used in our invention is a No. 12 B. W. G. galvanized steel wire in which the steel contained approximately 0.41% of carbon, approximately 0.21% of manganese, and less than 0.01% of silicon. A sample of this wire was hot-galvanized after being annealed, and showed a D. C. resistivity of approximately 5360 ohms per mile-pound, and a tensile strength of approximately 74,000 pounds per square inch. Another sample of this wire was hot-galvanized after receiving a heat-treatment and some cold drawing, and showed a D. C. resistivity of 5460 ohms per mile-pound, and a tensile strength of approximately 135,000 pounds per square inch.

Another example of carbon-steel conductor used in our invention is a No. 12 B. W. G. galvanized wire in which the steel contained approximately 0.35% of carbon, approximately 0.20% of manganese, and approximately 0.10% of silicon. A sample of this wire was hot-galvanized after being annealed, and showed a D. C. resistivity of approximately 6000 ohms per mile-pound, and a tensile strength of approximately 72,500 pounds per square inch. Another sample of this wire was hot-galvanized without being annealed, and showed a D. C. resistivity of approximately 6070 ohms per mile-pound, and a tensile strength of approximately 120,000 pounds per square inch.

By building an overhead transmission line of a carbon-steel conductor (coated or uncoated) conforming to the above requirements, it is possible to have both high tensile strength and high electrical conductivity. Such a transmission line

is of value for both alternating and direct currents, and for the transmission of electric power as well as of telephone, signal, and telegraph currents.

It is also advantageous for ground wires, shield wires, messenger cables, catenary supports, etc.; and either as a single wire or in a stranded cable. But it is of special advantage for the transmission of relatively high-frequency currents, such as those used in telephonic transmission; where the frequency is voice frequency, of the order of 100 to 3000 cycles per second, and the currents are usually small, not exceeding about 50 milliamperes.

We claim as our invention:

15

1. An overhead electric transmission line, comprising a carbon-steel conductor which is to carry current and which contains at least 0.25% of carbon and not in excess of 0.30% of manganese.

2. An overhead electric transmission line, comprising a hypoeutectoid carbon-steel conductor which is to carry current and which contains at least 0.25% of carbon and not in excess of 0.30% of manganese.

3. An overhead electric transmission line, comprising a carbon-steel conductor which is to carry current and which contains at least 0.25% of carbon, not in excess of 0.30% of manganese, and not on excess of 0.15% silicon.

4. An overhead electric transmission line, comprising a hypoeutectoid carbon-steel conductor which is to carry current and which contains at least 0.25% of carbon, not in excess of 0.30% of manganese, and not in excess of 0.15% silicon.

FRANK F. FOWLE. 35  
FREDERICK M. CRAPO.

#### CERTIFICATE OF CORRECTION.

Patent No. 2,019,447.

October 29, 1935.

FRANK F. FOWLE, ET AL.

It is hereby certified that error appears in the printed specification of the above numbered patent requiring correction as follows: Page 1, second column, line 26, after "and" insert are; and line 50, for "extra" read extra-high; page 3, first column, line 6, for "0,21%" read 0.21%; and second column, line 29, claim 3, for "on" read in; and that the said Letters Patent should be read with these corrections therein that the same may conform to the record of the case in the Patent Office.

Signed and sealed this 21st day of January, A. D. 1936.

Seal)

Leslie Frazer  
Acting Commissioner of Patents.